

## UNITED STATES PATENT OFFICE

2,406,823

## BITUMINOUS EMULSIONS

Joseph E. Fratis, Berkeley, and Eugene H. Oakley,  
El Cerrito, Calif., assignors to American  
Bitumuls Company, San Francisco, Calif., a  
corporation of Delaware

No Drawing. Continuation of application Serial  
No. 262,566, March 17, 1939. This application  
July 26, 1941, Serial No. 404,196

6 Claims. (Cl. 252—311.5)

1

The present invention pertains to aqueous bituminous emulsions and more particularly to emulsions of the fluid, quick-breaking penetration type.

It has previously been disclosed by Montgomerie, United States Patent No. 1,643,675, and by Braun, United States Patent No. 1,737,491, that asphaltic residues derived from certain petroleum crude oils, such for instance as those from Mexico, contain a proportion of saponifiable material which when the molten asphalt is dispersed in hot dilute aqueous caustic alkali solution reacts with the caustic to form an emulsifier in situ that is effective to produce an emulsion of unique and highly desirable characteristics. Such emulsions, which are generally referred to as "quick-breaking" or "penetrating" emulsions are now widely used in the construction and repair of roads and in various other important industrial operations. They are perfectly stable for long periods in storage but have a high and substantially instantaneous demulsibility when contacted with rock aggregates or other mineral or solid surfaces. They usually contain from 50 to 60% of dispersed bitumen and yet they are surprisingly fluid, having at ordinary temperatures a fluidity comparable to that of a light lubricating oil.

It is, however, now widely recognized that not all petroleum asphalts as regularly produced will emulsify by the simple method of dispersion in hot dilute alkaline solutions. This has usually been assumed to be due to a deficiency of acids or, more broadly, saponifiable ingredients in the asphalt. We have found that while this is probably the correct explanation in some cases it is not generally applicable since there are many asphalts having a relatively high content of free natural acids or saponifiable material which are nevertheless not emulsifiable by the Montgomerie method. On further studying these asphalts we have discovered that in order to produce a quick-breaking emulsion of the Montgomerie type it is not only necessary that the asphalt contain a certain minimum quantity of acids but also that the acids shall bear a certain molecular relation to the asphalt. On the basis of this discovery we have found it possible, as will be hereinafter fully explained, to so adjust and regulate the quantity and nature of the saponifiable petroleum ingredients in an asphalt that substantially all of those which do not, as ordinarily produced, emulsify or which form only poor emulsions by the Montgomerie method may be made to give quick-breaking emulsions that are entirely satisfactory for the usual commercial uses.

2

It is the broad object of this invention to so adjust the acid content of a petroleum asphalt that it will readily emulsify when dispersed in molten condition in a hot dilute aqueous solution of caustic alkali and will thereby produce a quick-breaking emulsion of the oil-in-water type that is stable in storage, of high bitumen content, high fluidity and high demulsibility on contact with mineral or other solid surfaces.

It is a more specific object of our invention to adjust the saponifiable ingredients of a petroleum asphalt both as to quantity and character for optimum emulsification when the asphalt is dispersed in a hot dilute alkaline solution.

It is a specific object of our invention to add to a petroleum asphalt organic acids, derived from petroleum, in quantity and character to co-operate with the acids naturally occurring in the asphalt in producing an emulsion of the quick-breaking type.

Another object of our invention is to make available for the production of quick-breaking emulsions large quantities of asphalts which have hitherto been unsuited for such use.

Other objects of our invention will be obvious from the description and discussion which follows.

The presence of organic acids in petroleum distillates and of both free acids and saponifiable substances such as acid anhydrides and possibly lactones in petroleum residue has long been known. The lower molecular weight acids occurring in the readily distillable fractions of crude petroleum are usually referred to as naphthenic acids while the acids of high molecular weight that are retained in the residual portion of the oil have been referred to by various writers as asphaltous or asphaltic acids. Very little, however, is actually known concerning these heavier acids and while there are some who believe that they differ only in degree from the naphthenic acids, the majority opinion appears to be that they differ in kind as well. Assuming that there is a difference in molecular structure between the acids of low and of high molecular weight, naturally occurring in petroleum as it comes from the earth, the transition is probably through several stages for each molecular series resulting in a range of overlapping types which would preclude the possibility of any simple method of separation or any definite point of division for classification. From a practical standpoint it is thus expedient to identify the natural petroleum acids with respect to their average molecular or equivalent weight and in the present connection that

practice will be adhered to except insofar as it may occasionally be convenient to refer more broadly to the acids below a somewhat arbitrarily chosen average equivalent weight of about 400 as "naphthenic" and those above as "asphaltic." 5

It is generally understood that in the preparation of an emulsion by the Montgomerie method the alkali metal salts of the acids occurring naturally in the asphalt are formed when the molten asphalt is dispersed in the hot aqueous alkaline solution and that these salts, produced as they are at the interface between the asphalt particles and the water continuous phase, serve as the emulsifiers which convert the dispersion into a true emulsion. In attempting to determine why asphalts that have a relatively high content of natural acids or saponifiable ingredients are, as above pointed out, nevertheless not satisfactorily emulsifiable by this method, we have found that the alkali metal salts of the natural petroleum acids of low molecular weight are quite soluble in water and relatively insoluble in oil and that as the molecular weight of the acid increases this preferential solubility shifts from the water side to the oil side so that the salts of acids in the asphaltic group are substantially insoluble in water and appreciably soluble in oil. We then found that in order to produce a satisfactory quick-breaking

10  
15  
20  
25  
30  
35  
40  
45  
50  
55  
60  
65  
70  
75  
80  
85  
90  
95

erably, also, they should have a molecular structure that is in general similar to the asphalt. In other words, salts of the acids occurring in or derived from a California "Midway" crude are more effective in emulsifying a "Midway" asphalt than are the same salts of acids from a totally different crude such as that from Michigan or Pennsylvania. For petroleum asphalts in general we have found that acids having an average equivalent weight between about 500 and 900 are usually most effective in the production of stable, fluid, quick-breaking emulsions by the Montgomerie method and further that such acids must be present to the extent of at least 1.00 to 1.50% by weight of the asphalt but should of course not be present in such large quantity as to result in an emulsion of low demulsibility and/or high settlement.

An investigation of asphalts from widely different sources has revealed a wide variation not only in the quantity but also in the character of the acids naturally present or available on saponification. The quantity may be from a few tenths of 1% to as much as 5% or more of the asphalt and the average equivalent weight from about 200 to well over 2,000. Pertinent analyses on a number of commercial asphalts from different localities are recorded in Table I.

Table I

| Source of asphalt             | Sample No. | Penetration at 77°F. | Melting point B & R °F. | Saponification number | Per cent total acids | Aver. equiv. wt. total acids | Emulsifiable Montgomerie method |
|-------------------------------|------------|----------------------|-------------------------|-----------------------|----------------------|------------------------------|---------------------------------|
| California (Midway).....      | 1024       | 124                  | 108                     | 1.40                  | 2.334                | 785                          | Yes.                            |
| Do.....                       | 1023       | 317                  | 93.5                    | 1.45                  | 2.528                | 690                          | Yes.                            |
| Do.....                       | 2214       | 200                  | 101.5                   | 1.56                  | 2.742                | 600                          | Yes.                            |
| Mexico.....                   | 2216       | 168                  | 105.5                   | 1.30                  | 1.298                | 535                          | Yes.                            |
| Wyoming.....                  | 2166       | 185                  | 104.5                   | 0.44                  | 1.236                | 1708                         |                                 |
| Oklahoma.....                 | 2217       | 173                  | 107                     | 0.40                  | 0.553                | 810                          |                                 |
| Arkansas.....                 | 2219       | 230                  | 101.5                   | 0.54                  | 1.520                | 475                          |                                 |
| Mid-Continent.....            | 2215       | 225                  | 105                     | 0.56                  | 0.638                | 524                          |                                 |
| Texas.....                    | 2218       | 99                   | 115.5                   | 0.42                  | 0.556                | 833                          |                                 |
| Montana.....                  | 2325       | 142                  | 107                     | 0.38                  | 0.925                | 1250                         |                                 |
| Bermudez Lake.....            | 2326       | 164                  | 106.5                   | 6.20                  | 2.377                | 585                          |                                 |
| California (Kern).....        | 2149       | 168                  | 102                     | 2.49                  | 3.338                | 672                          | Yes.                            |
| California (Mt. View).....    | 2027       | 182                  | 113                     | 0.41                  | 1.744                | 1586                         |                                 |
| California (Casmalia).....    | 1928       | 126                  | 111                     | 2.75                  | 3.158                | 703                          | Yes.                            |
| Mexico.....                   | 2338       | 77                   | 124                     | 1.02                  | 1.077                | 637                          | Yes.                            |
| Do.....                       | 2337       | 70                   | 124.5                   | 0.85                  | 1.062                | 878                          | Yes.                            |
| Do.....                       | 2340       | .....                | .....                   | 0.70                  | 0.844                | 1418                         | Almost.                         |
| California (Mid) treated..... | 2171       | 238                  | 98.5                    | 0.44                  | 2.320                | 1560                         |                                 |
| Mexico.....                   | 2357       | 157                  | 110                     | 1.15                  | 1.062                | 800                          | Yes.                            |

emulsion the acids present or liberated in an asphalt on saponification must form alkali salts that have the proper solubility relation in water and oil. If these salts are too water soluble they are withdrawn completely into the aqueous phase and such emulsion as may be formed will tend to have the characteristics of a conventional "soap-type" emulsion, in which a common fatty acid soap such as sodium oleate is employed as the emulsifier, rather than the high fluidity and quick-breaking characteristics necessary in a penetrating emulsion. On the other hand, if they are too insoluble in water they tend to be held in the oil phase and are not drawn into the interface to an extent or in a manner to effect emulsification.

While it is by no means easy to say specifically what the character of the acids must be in order that their alkali salts will have the proper solubility relations to function as effective in situ emulsifiers, it has been found that in general they should be of about the same average molecular weight as the asphalt they are to emulsify. Pref-

55  
60  
65  
70  
75  
80  
85  
90  
95

It will be observed that all of the asphalts, recorded in the above Table I, that contain acids of an average equivalent weight between 500 and 900 in an amount above about 1% were found to be emulsifiable by the Montgomerie method. The asphalts recorded which were not emulsifiable by this method deviate in one or more of three ways from these limits as follows:

Samples Nos. 2027, 2166 and 2171 contain more than the minimum 1% of acids but they are substantially above the optimum average equivalent weight; sample No. 2219 contains more than 1% of acids but they are below the optimum average equivalent weight; samples Nos. 2215, 2217 and 2218 contain acids of the optimum average equivalent weight but in amount less than 1%; and sample No. 2325 contains less than 1% of acids having an average equivalent weight above the optimum range. We have found that when the average equivalent weight of the acids in samples Nos. 2027, 2166, 2171 and 2325 is adjusted downward by the addition of acids of substantially lower equivalent weight than those naturally oc-

curing, as for instance through the addition of acids having an average equivalent weight from about 400 to 700, the asphalts are rendered readily emulsifiable. Likewise, when the acid content of samples Nos. 2215, 2217 and 2218 is brought above the minimum 1% by the addition of acids having an average equivalent weight within the optimum range from 500 to 900 and when the average equivalent weight of the acids in sample No. 2219 is raised by the addition of similar acids, all of these samples are easily emulsified when dispersed in hot alkali solution.

While, as hereinabove indicated, the average equivalent weight of the naturally occurring acids in a petroleum asphalt for its optimum emulsification lies between about 500 and 900, we have found that it is not always necessary when adjusting a very high average equivalent weight downward through the addition of substantially lighter acids to come within this range since a reduction to about 1200 or below is frequently adequate to give an asphalt of satisfactory emulsifying characteristics.

It would thus appear that the optimum average weight of asphaltic acids for the production of satisfactory emulsions by the Montgomerie method depends somewhat upon the distance apart of the extremes comprehended by the average. When that distance is relatively great, as for instance from 400 to 1800 or above, satisfactory emulsions are produced when the weighted average equivalent weight is reduced to only about 1200, whereas when the acids cover a narrower range a weighted average between about 500 and 900 will usually be more desirable.

The foregoing principles may be further illustrated by the following examples:

*Example No. 1*

Wyoming asphalt, sample No. 2166, which will be seen by reference to Table I to contain 1.236% of acids of 1708 average equivalent weight, was found not to give an emulsion when dispersed in hot aqueous 0.05% normal sodium hydroxide solution. When 0.28% of acids from a California Midway crude having an average equivalent weight of 666 was added, giving a product containing 1.516% of acids having a weighted average equivalent weight of 1510, more tendency toward emulsification was shown but still no satisfactory emulsion could be produced. When, however, 1.27% of these same acids was added to the asphalt, giving a product containing 2.506% of acids having a weighted average equivalent weight of 1177, a stable fluid emulsion of high demulsibility was produced on dispersion in dilute caustic solution. When a still greater amount, 5.3%, of the same acids was added to the same asphalt, giving a product containing 6.536% of total acids having a weighted average equivalent weight of 863, its emulsibility was still further enhanced but the emulsion formed showed excessive settlement on standing and a low demulsibility.

*Example No. 2*

To California asphalt sample No. 2027, which contained 1.744% of acids having an average equivalent weight of 1586 and which was not emulsible by the Montgomerie method, was added 0.1% of acids from Midway crude having an average equivalent weight of 357. The total acids in the asphalt then amounted to 1.844% having an average equivalent weight of 1535. While the product showed some tendency to emulsify, it

still would not produce a satisfactory emulsion. When, however, 1.0% of the same acids was added, giving a product having 2.744% of acids of average equivalent weight 1140, an entirely satisfactory emulsion could be produced.

*Example No. 3*

2.0% by weight of acids from California crude having an average equivalent weight between 406 and 460 when added to Texas asphalt sample 2218 gave a product of good emulsibility. When, however, acids having an average equivalent weight of 273 were added to this same asphalt in quantities from 1.0% to 10.0%, no satisfactory emulsion could be produced.

For determining the acid content of an asphalt we have found the following simple method entirely satisfactory: 30 grams of asphalt are dissolved in 60 cc. of a light petroleum thinner, known in the trade as "10-P" thinner, 300 cc. of 95% ethyl alcohol and 5 cc. of water containing 2.4 grams of pure sodium hydroxide are added and the mixture then boiled under a reflux condenser for one hour, after which water sufficient to reduce the alcohol concentration to 80% is added through the condenser, the mixture cooled and transferred to a separatory funnel wherein it is allowed to stand in a warm place over night. The two layers are separated and the asphalt-petroleum thinner layer washed with 80 cc. of 95% alcohol. The main alcoholic extract is washed with three successive 100 cc. portions of petroleum ether, the petroleum ether washes are combined in a separatory funnel, the 80 cc. portion of alcohol previously used to wash the asphalt layer is added thereto together with 20 cc. of water and the mixture vigorously shaken. On separation the alcoholic layer is united with the main body of alcoholic extract. The petroleum acids may then be separated from this extract by acidifying with hydrochloric acid and dilution with water, their quantity determined by weighing and their average equivalent weight determined by titration or they may be separated roughly into groups by successively extracting the alcoholic solution with appropriate solvents of progressively varying solvent power.

Acids which may be used for adjusting the acid content of asphalts in accordance with the principles of our invention, as hereinabove set forth, may be derived from petroleum in a number of ways. One readily available source of such acids is from the still bottoms produced when a heavy lubricating oil fraction is distilled over caustic soda for the reduction of organic acidity. Such still bottoms contain the sodium salts of the petroleum acids which may be liberated by acidification with a mineral acid, collected and redistilled if necessary to segregate the acids of higher equivalent weight useful in the practice of our invention.

Another source of almost unlimited quantities of natural petroleum acids for use in adjusting the acid content of asphalts is through the simple caustic alkali or alcoholic caustic alkali extraction of petroleum residua, road oils, fuel oils and asphalts which are not intended for emulsification. The acids are, of course, liberated by acidification and collected in any appropriate manner.

Satisfactory acids for our purpose may also be derived from various heavy petroleum fractions that have been subjected to very mild oxidation such that the acids produced are largely simple carboxylic acids rather than the acids of higher oxygen content which are usually referred to as

oxy-acids. For instance, it has been found that the acids which may be recovered from a sample of heavy lubricating oil after use in regular service in an automobile engine are entirely satisfactory for adjusting the acid content of an asphalt as hereinabove described. The carboxylic acids produced by air blowing a heavy cylinder stock at about 300 to 400° F. for several hours have also been found effective in this connection.

While the adjustment of the acid content of an asphalt as contemplated by our invention will usually be by the addition of petroleum acids from an external source, it is conceivable that it might under certain circumstances be more desirable to arrive at the desired adjustment by extracting either the very heavy or the very light acids or by the extraction of all the acids with the subsequent return of the desired portions thereof. Any such operation will be readily seen to be consistent with the principle hereinabove set forth. Still another method of arriving at our ultimate result may be possible with an asphalt which is found to be unsatisfactorily emulsifiable, due to an excess of low equivalent weight acids, since we have found that on moderate heating for considerable periods of time the acidic constituents of an asphalt are quite readily polymerized without, however, having their acidic nature appreciably altered. This fact is illustrated by a comparison of samples Nos. 1024 and 2171 of Table I. Sample No. 2171 was prepared by moderately heating an asphalt which was originally comparable to that of sample No. 1024. It will be noted that while the total acid content remained substantially the same, the average equivalent weight of the acids was increased from about 800 to 1560, and while in this specific instance the asphalt was rendered unemulsifiable by the increase in equivalent weight, a similar doubling of the equivalent weight of acids in the range of 360 or below would throw them into the range of 500 to 900 which has been found to give desirable emulsification.

Throughout the foregoing discussion we have referred to the caustic solutions suitable for producing quick-breaking emulsions of the Montgomerie type only as "dilute aqueous" solutions. It will be understood that the several caustic alkalies are substantial equivalents in this use. The concentration may vary somewhat depending on the particular asphalt to be emulsified and the specific conditions under which emulsification is to be effected but will usually be within the range between 0.05 and 0.10 normal.

When in the foregoing discussion and in the appended claims the "acid content" of an asphalt is referred to without further characterization, it will be understood to mean the total available acid whether in the form of free acid or whether in a combination from which it may be liberated on contact with hot caustic solution.

This application is a continuation of application Serial No. 262,563, filed March 17, 1939.

Having now fully described our invention which consists in adjusting the acid content of an asphalt for optimum emulsification, to give a stable, fluid, quick-breaking emulsion when dispersed in hot dilute aqueous caustic alkali solution, we claim:

1. A method of producing an asphalt which is emulsifiable in hot, dilute aqueous caustic soda solution from an asphalt which is not so emulsifiable, which comprises adjusting the petroleum acid content of the asphalt not so emulsifiable,

without otherwise substantially changing the composition of the asphalt, so as to produce an asphalt having at least about 1% and not more than about 3% by weight, based on the asphalt, of petroleum acids having an average molecular weight of about 500 to 1200, said petroleum acid content being adjusted to an amount sufficient only to produce an asphalt which is emulsifiable in hot, dilute aqueous caustic soda solution to form an emulsion which breaks quickly on contact with aggregate.

2. In a process wherein asphalt which is not emulsifiable in hot, dilute aqueous caustic soda solution is rendered emulsifiable in hot, dilute aqueous caustic soda solution by incorporating in the asphalt a saponifiable material, the improvement which comprises adding to the asphalt sufficient substantially unadulterated petroleum acids to cause the asphalt to contain at least about 1% and not more than about 3% by weight, based on the asphalt, of petroleum acids having an average molecular weight of about 500 to 1200, the amount of petroleum acids so added being sufficient only to produce an asphalt which is emulsifiable in hot, dilute aqueous caustic soda solution to form an emulsion which breaks quickly on contact with aggregate.

3. A method of producing an asphalt which is emulsifiable in hot, dilute aqueous caustic soda solution from an asphalt which is not so emulsifiable and which has a petroleum acid content above about 1% by weight based on the asphalt and of average molecular weight exceeding 1200, which comprises removing from said asphalt not so emulsifiable sufficient acids of high molecular weight to produce an asphalt having about 1% to 3% by weight based on the asphalt of acids having an average molecular weight between about 500 and 1200, the amount of petroleum acids so removed being sufficient only to produce an asphalt which is emulsifiable in hot, dilute aqueous caustic soda solution to produce an emulsion which breaks quickly on contact with aggregate.

4. A method of producing an asphalt which is emulsifiable in hot, dilute aqueous caustic soda solution from an asphalt which is not so emulsifiable and which has a petroleum acid content above 1% by weight based on the asphalt and of average molecular weight below 500, which comprises subjecting the asphalt to heat treatment sufficient to produce an asphalt having about 1% to 3% by weight based on the asphalt of petroleum acids having an average molecular weight of about 500 to 1200, said heat treatment being sufficient only to produce an asphalt which is emulsifiable in hot, dilute aqueous caustic soda solution to produce an emulsion which breaks quickly on contact with aggregate.

5. The method of claim 1, in which the petroleum acid content of the asphalt is adjusted so as to produce an asphalt having at least about 1% and not more than about 3% by weight, based on the asphalt, of petroleum acids having an average molecular weight of about 500 to 900.

6. The improvement of claim 2, in which there is added to the asphalt sufficient substantially unadulterated petroleum acids to cause the asphalt to contain at least about 1% and not more than about 3% by weight, based on the asphalt, of petroleum acids having an average molecular weight of about 500 to 900.